

# UNITED STATES PATENT OFFICE.

JOHN L. COX, OF PHILADELPHIA, PENNSYLVANIA.

## PROCESS OF HEAT-TREATING AND HARDENING PROJECTILES.

1,407,255.

Specification of Letters Patent. Patented Feb. 21, 1922.

No Drawing. Application filed July 16, 1919, Serial No. 311,325. Renewed November 29, 1920. Serial No. 427,232.

*To all whom it may concern:*

Be it known that I, JOHN L. COX, a citizen of the United States, residing at Philadelphia, county of Philadelphia, and State of

5 Pennsylvania, have invented a new and useful Improvement in Processes of Heat-Treating and Hardening Projectiles, of which the following is a full, clear, and exact description.

10 In the manufacture of armor piercing shot and shell the necessity of combining in a projectile formed of a single block of metal a hard but not brittle head with a relatively soft and very tough body is well recognized, 15 and projectiles having in degree such characteristics have hitherto been manufactured.

Known processes of manufacture still leave much to be desired in obtaining and combining these desirable and apparently contradictory qualities; moreover, a considerable proportion of projectiles that have been subjected to recognized methods of heat treatment designed to produce the desired result fail when subjected to the rigorous ballistic 25 tests which they must pass to be accepted.

It is the object of my invention to manufacture a projectile which will possess to a maximum degree the qualities above mentioned, and by a process which will minimize 30 the likelihood of producing any defects or weaknesses which might endanger acceptance or, later, cause spontaneous rupture in storage.

By my process a projectile is produced 35 having a point characterized by a high degree of hardness, progressively decreasing through the head toward its junction with the body, and a body sufficiently soft to permit machining yet so tough that it will not 40 break upon impact; moreover the process is one wherein the danger of cracking during treatment is minimized, and all danger of the shell cracking in storage after delivery is removed.

45 In the heat-treatment of steel certain laws are more or less well known, but there are many conceivable ways of applying them to heat treating processes, and there is always the danger that while some of these laws may 50 be regarded others might be overlooked or ignored.

The laws that I have more especially borne in mind in the development of my process are the following:

55 1. On heating, at the  $Ac_1$  point the previ-

ously existing cell boundaries of the steel begin to disappear as the solution commences, but are not entirely gone until the  $Ac_3$  point is reached.

2. At the  $Ac_1$  point a new cell structure begins to form and to grow larger as the temperature increases.

3. There is a cell size corresponding roughly to any given temperature above the  $Ac_1$  point, long maintenance at that temperature tending rather to increase the thickness of the cell boundaries than to increase the cell size.

4. To acquire, on sudden cooling, the maximum hardness permitted by its chemical composition steel must first be heated to or above the  $Ac_3$  point.

5. The degree of final hardness is dependent upon the speed of the quench.

6. Steel raised to a temperature much in excess of the  $Ac_3$  point tends to become coarse in grain and brittle.

7. The power of hardening once acquired by steel on heating is not lost, on slow cooling, until the  $Ar_1$  point is passed.

8. Sudden cooling from below the  $Ar_1$  point theoretically will not produce hardening but the steel will be in the same soft or annealed state that it would be had it been slowly cooled.

9. It is much less well known that on heating, sudden cooling from a point within a substantial, but limited, range below the  $Ac_1$  point as experimentally determined, may produce a distinct degree of hardening and notable loss of toughness; while sudden cooling from a temperature too far below the  $Ac_1$  point to produce this effect will impart a degree of toughness superior to that resulting from a slow cooling from the same or somewhat higher temperature.

10. It is also known to but few that the  $Ac_1$  and  $Ac_3$  points are not fixed points for any particular composition but vary with the degree of grain-refinement of the steel, being 11 lower as the grain of the steel is finer.

I shall not herein describe the process of melting the steel and casting, or casting and forging, the projectile.

12 After production, the projectile, as it comes from the forge at a temperature substantially above the  $Ac_3$  point, may be cooled slowly until below the  $Ar_1$  point; but preferably, in order to arrest the growth of the cell walls, the projectile may be cooled suddenly to ap-

oximately the  $Ar_1$  point, and thereafter cooled more slowly.

The next procedure is to refine the grain and soften for preparatory machining. The projectile is raised to a temperature above the  $Ac_3$  point, and maintained at that temperature long enough to allow complete solution of the microscopic constituents. It may then be cooled with extreme slowness, to below the  $Ar_1$  point; but preferably, in order to retain as fine a grain as possible, it is cooled rapidly to below the  $Ar_1$  point, then repeated to below the  $Ac_1$  point, maintained at that temperature for a time, and allowed to cool slowly or rapidly.

The projectile is now in the best possible condition for further heat-treatment, and is, moreover, in an extremely soft condition permitting easy preparatory machining.

After the preparatory machining the projectile is then still further grain-refined. It is heated to about  $130^\circ$  C. above the  $Ac_3$  point, maintained there a proper length of time to insure complete solution,—the time pending upon its size—is rapidly withdrawn from the furnace and quenched in water until well below the  $Ar_1$  point throughout its entire mass.

Depending upon the calibre of the projectile, this step is applied one or twice. The projectile is next heated to a temperature of about  $75^\circ$  C. above the  $Ac_3$  point, similarly maintained at that temperature and similarly quenched.

It is to be observed that in both cases the temperatures are higher than the theoretically correct points but are given in practice to hasten the necessary molecular transformations, while the time is not to be long enough to cause appreciable grain growth.

The projectile is next heated to a temperature about  $75^\circ$  C. below the  $Ac_1$  point and quenched for a few minutes in warm water, necessary care being taken to remove the projectile from the water before cracking occurs. The projectile is then allowed to cool to atmospheric temperature.

If the composition of the projectile has been properly chosen and all steps of melting, forging, and the heat-treatment described above properly applied, the projectile will be in the condition of maximum hardness throughout, and soft enough ready to allow machining to finish sizes, should this step not already have been applied. It is generally advisable not to finish the band score at this stage.

The projectile being ready for its final hardening I first preliminarily heat it in a furnace to a temperature below the  $Ac_1$  point, and then heat the head of the projectile, and at least the forward part of the body, to above the  $Ac_3$  point of the steel. This is best done by holding the projectile by its base and immersing the head and all

or nearly all of the body in a bath of melted lead raised to the necessary temperature. Bearing in mind that the head is solid and the body hollow, and that, therefore, the greater thickness of metal is in the head, it is best at first to immerse only the point and head, or (say) that part of the projectile forward of the tip of the cavity, and, after they have acquired substantially the temperature of the lead then to submerge all or nearly all of the body.

If the projectile be held by a mechanism operating in the bore it should be possible to submerge practically the entire body. If the handling mechanism holds the projectile by the exterior near the base it should be possible to submerge the projectile to about the line of the band score.

After the projectile has been heated up to the prescribed temperature and been maintained at that temperature for a sufficient length of time for the full development of its capacity for hardening it is withdrawn and quenched in a suitable liquid or liquids, for which purpose I prefer to employ a spray of water under pressure. The spraying of the liquid is continued until the temperature of the projectile approaches the normal,—say below  $120^\circ$  C.

As soon after the hardening as possible, I slowly warm the projectile, conveniently by immersion in hot water, and after it has acquired the temperature of the water, transfer it to a bath of heated oil in which it is kept for a length of time sufficient for the practical completion of the drawing effects of that temperature. The exact temperature and time of the drawing depend somewhat upon the composition and calibre of the projectile, the first being not over  $200^\circ$  and generally not over  $150^\circ$  C. nor under  $95^\circ$  C., and the latter generally not less than six hours.

By this step the mineralogical hardness of the projectile is very slightly reduced but the loss in hardness is far more than offset by the increase in toughness of the slightly tempered steel and by the release in large part of the stresses set up in hardening. Properly applied, this step has proved a complete cure for the serious losses which formerly occurred through spontaneous rupture of finished projectiles,—even months after their delivery.

After cleaning the projectile from oil I then heat the body, from the base end, to about  $70^\circ$  C. below the  $Ac_1$  point of the steel. This is best done by holding the projectile by the head and immersing the body, either gradually or suddenly, in a bath of lead heated to the necessary temperature. The depth of this immersion and the temperature of the lead will vary somewhat with the precise results that are sought to be obtained. Generally, it is best first to immerse the projectile to about the rear edge of the band score,

in order slightly to warm the projectile and reduce the risk of cracking, then further to immerse it to a depth of about two-thirds of the body length for a time long enough to 5 thoroughly draw the hardness from that portion of the projectile. It may sometimes be then further immersed for a shorter period of time as far as the forward edge of the bourrelet and there maintained until the 10 hardness of the head remaining outside of the lead has been drawn to nearly the desired degree.

I then remove the projectile from the lead and quench the body in a spray of water under pressure, care being taken, preferably, to leave a narrow zone of incandescent metal 15 above the line of the spray, and therefore unquenched by it, to avoid danger of cracking the head.

20 As soon as the body of the projectile has reached normal temperature, which, in such a spray as I have described, will occur in a very few minutes, I invert the projectile and place it point downwards in a shallow 25 bath of water to prevent the further softening of the point, which would otherwise occur through the transmission of heat from the heavier section of the head.

The effect of the above treatments is to 30 impart to the head the maximum degree of hardness at the point, and a diminishing degree of hardness towards the rear without impairing the fine-grained structure of the steel, while imparting to the body the 5 maximum degree of toughness, and a sufficient degree of softness to enable it to be readily machined if desired, as, for instance, for the attachment of the band.

While it is true that the elevation of the 40 temperature of the rear of the head in the final heating operation due to the conductivity of the metal modifies somewhat its hardness, the modification is such that it would be desirable to take special means to 45 obtain it; that is, the objectionable brittleness necessarily associated with extreme hardness is largely eliminated where maximum hardness is not necessary, but there is secured a maximum degree of hardness consistent with the reduction of brittleness to 50 the desired extent. However, the amount of heat transmitted from the head to the point during the cooling of the head must be restricted to prevent diminution of the 55 hardness of the point.

As it is usually dangerous to quench the whole projectile after the heating of the body, in that the projectile is likely to crack, I prefer, as described above, to quench substantially all the body and subsequently to 60 submerge the point in water, thereby holding down the temperature of the point.

I wish it to be understood that there is no clear line of demarcation between the 65 hard and tough portions of the projectile;

on the contrary there is between the hard point and the tough body the major portion of the head, shading in hardness from the point toward the body, which is not as hard as the point nor as tough as the major 7 portion of the body.

While I have referred to the projectiles to which my process is applied as steel projectiles, it is not intended that the process shall be limited to projectiles consisting of 7 simple carbon steel only. I mean to include projectiles of steel alloyed with other metals,—various compositions of said alloys being well known and successfully used.

The exact temperatures corresponding 8 to the  $Ac_1$ ,  $Ac_3$  and  $Ar_1$  points will vary with the composition and physical structure of the steel and cannot be definitely stated; but these points are well known to metallurgists and practical steel workers and are 8: more informative than the specification of exact temperatures. Instruments of a number of forms exist for their accurate determination.

Where, in the specification, I use the term 90 "slow cooling", I mean to imply that the rate of cooling, as compared with free cooling in air, is retarded. Where "quick cooling" is specified, I mean to include not only quenching in liquid, but also freely cooling 95 in air, the latter operation being rapid relatively to retarded cooling. By "sudden cooling" or "quenching" I mean to imply the use of a liquid to accelerate cooling.

Having now fully described my invention, 10 what I claim and desire to protect by Letters Patent is:

1. The process of heat treating projectiles which comprises suddenly cooling the projectile from a temperature substantially 10 above the  $Ac_3$  point to a temperature not higher than approximately the  $Ar_1$  point, thus arresting the growth of the cell walls, then cooling relatively slowly, then heating to and above the  $Ac_3$  point, then cooling 11 quickly to below the  $Ar_1$  point, then heating to below the  $Ac_1$  point, then cooling, then subjecting the projectile to a plurality of grain-refining operations in one of which the projectile is heated to substantially 11: above the  $Ac_3$  point and cooled suddenly to below the  $Ar_1$  point and in a later one of which the projectile is heated to a lower temperature but still above the  $Ac_3$  point and similarly cooled below the  $Ar_1$  point, 120 then heating to below the  $Ac_1$  point and quenching and cooling to atmospheric temperature, then heating the head and at least the forward part of the body to above the  $Ac_3$  point, suddenly cooling by quenching, 125 drawing the temper of the hardened part of the projectile at a temperature below 200° C., heating the body of the projectile from the base end to below the  $Ac_1$  point, quenching the last named part of the pro- 130

tile, and then placing the point of the projectile in a cooling medium to preserve the desired degree of hardness of the point.

2. The process of heat treating projectiles which comprises suddenly cooling the projectile from a temperature substantially above the  $Ac_3$  point to a temperature not higher than approximately the  $Ar_1$  point, thus arresting the growth of the cell walls, then cooling relatively slowly, then heating above the  $Ac_3$  point, then cooling quickly

below the  $Ar_1$  point, then heating to below the  $Ac_1$  point, then cooling, then subjecting the projectile to a plurality of grain-refining operations in one of which the projectile is heated to substantially above the  $Ac_3$  point and cooled suddenly to below the  $Ar_1$  point and in a later one of which the projectile is heated to a lower temperature but still above the  $Ac_3$  point and similarly cooled below the  $Ar_1$  point, then heating to below the  $Ac_1$  point and quenching and cooling to atmospheric temperature, and then subjecting the projectile to a hardening treatment.

3. The process of heat treating projectiles which comprises initially suddenly cooling the projectile from a temperature substantially above the  $Ac_3$  point to a temperature not higher than approximately the  $Ar_1$  point, thus arresting the growth of the cell walls, and thereafter cooling relatively slowly, then subjecting the projectile to successive heating and cooling to refine the grain and soften for preparatory machining, then subjecting the projectile to a succession of heating and cooling treatments to further refine the grain and impart to the projectile a tough condition known as fibrous, and then subjecting the projectile to a final hardening treatment.

4. The process of heat treating projectiles which comprises initially suddenly cooling the projectile from a temperature substantially above the  $Ac_3$  point to a temperature not higher than approximately the  $Ar_1$  point, thus arresting the growth of the cell walls, and thereafter cooling relatively slowly, and then refining the grain and softening for preparatory machining by heating the projectile to above the  $Ac_3$  point of the steel, then cooling quickly to not approximately above the  $Ar_1$  point, then reheating to below the  $Ac_1$  point and then cooling.

5. The process of heat treating projectiles which comprises first refining the grain and imparting a tough fibrous condition to the steel by subjecting the projectile to heating and cooling to refine the grain and soften for preparatory machining, then heating to above the  $Ac_3$  point and quenching, heating to below the  $Ac_1$  point and again quenching, and afterward subjecting the projectile to a hardening treatment.

6. The process of heat treating projectiles

preparatory to final hardening which comprises heating the projectile above the  $Ac_3$  point and quickly cooling to a temperature below the  $Ar_1$  point, reheating to below the  $Ac_1$  point and cooling, thereby refining the grain and softening for preparatory machining, heating to above the  $Ac_3$  point and quenching to below the  $Ar_1$  point, and heating to below the  $Ac_1$  point and quenching, thereby imparting a tough fibrous condition to the steel.

7. The process of heat treating projectiles which comprises subjecting the projectile to heating and cooling to soften for preparatory machining and then subjecting the projectile to a plurality of grain-refining operations in one of which the projectile is heated to substantially above the  $Ac_3$  point and cooled suddenly well below the  $Ar_1$  point and in a later one of which the projectile is heated to a lower temperature but still above the  $Ac_3$  point and similarly suddenly cooled below the  $Ar_1$  point.

8. The process of hardening heat-treated projectiles which comprises heating the head and at least the forward part of the body to above the  $Ac_3$  point of the steel, quenching the projectile in a suitable cooling medium so as to produce maximum hardness of the steel, heating the body of the projectile from the base end to below the  $Ac_1$  point of the steel, while maintaining the point out of contact with the heating medium, and quenching only the body of the projectile in a suitable cooling medium so as to produce maximum toughness of the body.

9. The process of hardening heat-treated projectiles which comprises heating the head and at least the forward part of the body to above the  $Ac_3$  point of the steel, suddenly cooling, heating the body of the projectile to below the  $Ac_1$  point of the steel and suddenly cooling the body, and, after substantial cooling of the body has occurred, bringing and holding the point of the projectile under the influence of a cooling medium until the whole projectile is cooled.

10. The process of hardening heat-treated projectiles which comprises heating the head and at least the forward portion of the body to above the  $Ac_3$  point of the steel while holding the projectile by the base, quenching the projectile in a suitable cooling medium, heating the body of the projectile to below the  $Ac_1$  point of the steel while holding the projectile by the head and maintaining the point out of contact with the heating medium, and quenching only the body in a suitable cooling medium.

11. The process of hardening heat-treated projectiles which comprises heating the head and at least the forward part of the body to above the  $Ac_3$  point, suddenly cooling, drawing the temper of the hardened part of the projectile at a temperature below

200° C., heating the body of the projectile from the base end to below the  $Ac_1$  point, and quenching the last named part of the projectile.

12. The process of hardening heat treated projectiles which comprises heating the head and at least the forward part of the body to above the  $Ac_3$  point of the steel, quenching the projectile in a suitable cooling medium so as to produce maximum hardness of the steel, immersing a part of the projectile from its base end in a heating medium, then after an interval immersing the projectile in said heating medium to a greater depth while maintaining the point out of contact with the heating medium, and then quenching the larger part of the heated portion of the projectile from the base forward while maintaining the point unquenched.
13. The process of heat treating projectiles which comprises heating the projectile to above the  $Ac_3$  point, then cooling, afterward heating to above the  $Ac_3$  point, then cooling suddenly, then heating to below the  $Ac_1$  point, then cooling, then heating the head and at least the forward part of the body to above the  $Ac_3$  point, suddenly cool-

ing by quenching, heating the body of the projectile from the base end to below the  $Ac$  point, and afterward placing the point of the projectile in a cooling medium to preserve the desired degree of hardness of the point.

14. The process of hardening heat treated projectiles which comprises heating the head and at least the forward part of the body to above the  $Ac_3$  point of the steel, quenching the projectile in a suitable cooling medium so as to produce maximum hardness of the steel, immersing a part of the projectile from its base end in a heating medium, then after an interval immersing the projectile in said heating medium to a greater depth while maintaining the point out of contact with the heating medium, and then quenching the larger part of the heated portion of the projectile from the base forward while maintaining above the cooling medium a narrow zone of incandescent metal to avoid cracking of the head.

In testimony of which invention, I have hereunto set my hand, at Philadelphia, Pa., on this 1st day of July, 1919.

JOHN L. COX.